

March 31, 1925.

1,531,784

C. W. HAZELETT

SHEET METAL

Filed Dec. 13, 1921

2 Sheets-Sheet 1



INVENTOR

Clarence W. Hazelett,  
By Davis & Macklin,  
ATTORNEYS

March 31, 1925.

1,531,784

C. W. HAZELETT

SHEET METAL

Filed Dec. 13, 1921

2 Sheets-Sheet 2



MOULD CAST  
SHEET  
100 DIAMETERS

FIG. - 7



ORDINARY  
ROLLED SHEET  
100 DIAMETERS

FIG. - 8



MOULD CAST  
100 DIAMETERS

FIG. - 9

INVENTOR  
C. W. Hazelett,  
By Park MacLean,  
ATTORNEY'S

Patented Mar. 31, 1925.

1,531,784

# UNITED STATES PATENT OFFICE.

CLARENCE W. HAZELETT, OF CLEVELAND, OHIO, ASSIGNOR, BY MESNE ASSIGNMENTS,  
TO THE CLEVELAND TRUST COMPANY, TRUSTEE, OF CLEVELAND, OHIO.

## SHEET METAL.

Application filed December 13, 1921. Serial No. 522,108.

*To all whom it may concern:*

Be it known that I, CLARENCE W. HAZELETT, a citizen of the United States, residing at Cleveland, in the county of Cuyahoga and State of Ohio, have invented a certain new and useful Improvement in Sheet Metal, of which the following is a full, clear, and exact description, reference being had to the accompanying drawings.

10 This invention relates to cast sheets of metals of the lower and medium melting temperatures, as distinguished from metals having high melting temperatures, such as steel. I have discovered that certain characteristics of thin cast sheet metal are coincident with results of greater economy of manufacture, greater strength, more uniform physical characteristics, and very much higher degree of resistance to corrosive actions.

Up to the time of the present invention steel metal in commercial use is manufactured almost entirely by rolling processes, although a small amount may be made by casting sheets of small area in molds. I have produced a metal resulting in the above and other advantages, and capable of being manufactured in large commercial quantities at an exceeding low cost, by a continuous casting process, resulting in a continuous strip of predetermined thickness and width, delivered at a high rate of speed. Such a process, adapted for making the sheet metal herein described, is fully disclosed and claimed in my copending application filed November 11th, 1920, Serial Number 423,309.

It is my intention to confine the present application entirely to my sheet metal. To 40 determine the characteristics of my sheet metal, as to its strength, acid resisting properties and other properties, comparison may be made with the characteristics of sheets formed by methods previously known and used.

To fully disclose this invention, I illustrate the characteristics of the crystalline structure, and describe its properties as embodied in sheets made of a certain lead alloy, and compare these properties and characteristics with those of rolled and cast sheets of the same alloy, made in the forms heretofore used. Therefore, in the drawings, Fig. 1, is a section perspective of a piece of my sheet metal considerably enlarged; Figs. 2, 3, 4

and 5 are reproductions of micro-photographs, taken after etching, illustrating the crystalline structure, progressively from one side of the sheet to the other and taken at right angles to the plane of the sheet, approximately in the position shown by the small circles with which each of these figures is connected; Fig. 6 is a reproduction of a micro-photograph taken after etching and in the same plane as the sheet at the side 60 on which Fig. 5 terminates; Fig. 7 is a reproduction of a micro-photograph of a sheet of similar thickness cast in a mold; Fig. 8 is a reproduction of a micro-photograph illustrating the structure of a rolled sheet; Fig. 9 is a similar reproduction of cast pig or ingot of the same alloy as the sheet illustrated in Figs. 1 to 6. The micro-photographs from which Figs. 7, 8 and 9 are taken are made at 100 diameters, as are the other 75 views 2 to 6.

My sheet metal is hereinafter more fully described in reference to the drawings and its particular novel characteristics are summarized in the claims.

The sheet embodying my invention and discovery has within the meaning of the appended claims and as above outlined, certain very marked novel features of crystalline structure. As at present successfully practiced, the results may be illustrated by an alloy in wide commercial use, for example, for storage battery plates, linings for acid tanks and other uses, and composed of 7 per cent antimony and 93 per cent lead. Variations of these proportions and other ingredients in similar alloys produce structural results quite like those illustrated in Figs. 1 to 6.

In Fig. 1, 10 designates a sheet being a representation of a small piece taken from a commercial sheet of my metal made in a continuous strip and enlarged to five diameters for clearness of illustration.

Discussing first, the crystalline structure 100 of sheets of this antimony lead, examination under microscope has disclosed that at one side of the sheet, it has a coarse crystalline structure while at the other side the crystals are comparatively small. This outstanding 105 feature is noticeable in my sheets made of various metals, and particularly when made by my process, described in the previously mentioned application. At one side of the sheet of metal, the crystalline structure is 110

similar to the normal crystalline structure of a cast piece of material with comparatively large crystals, while at the other side of the sheet are fine small crystals, and the size 5 from one side to the other grows progressively smaller with considerable uniformity. In this discussion, I am referring to sheets from a few thousandths of an inch in thickness up to sheets of one eighth of an inch or 10 somewhat greater, although it is to be understood I do not wish to limit my invention to particular thickness of the sheet, other than to consider its scope as relating to comparatively thin sheets of material.

15 Illustrating this decreasing of the size of the crystals from one side of the sheet to the other, we may refer to Figs. 2, 3, 4 and 5, the circle of vision of which is illustrated to define its position with relation to the sheet 20 by the circles 2<sup>a</sup> 3<sup>a</sup>, 4<sup>a</sup> and 5<sup>a</sup>, respectively. Fig. 2 is taken to include the upper edge of the sheet, that is from the upper surface into the metal, say one fourth of its thickness. It shows the coarser crystals. It can be 25 noted that the crystalline structure reproduced in Fig. 3, is somewhat finer than that of Fig. 2. Fig. 4 which is taken still farther from the upper side of the sheet 30 is still smaller than that of Fig. 3 and the size of the crystals is very noticeably smaller than those of Fig. 2 at the top of the metal sheet. In this view the crystals grow noticeably 35 smaller from the upper part of Fig. 4 to the lower part, while Fig. 5 which includes the lower edge of the sheet shows the very fine crystalline structure at the lower side of the sheet. The upper part of this Figure 5 (which includes the same zone as the lower part of the Figure 4) shows a crystal formation 40 substantially the same as Fig. 4 at its lower side.

The relationship of the crystals, one to another, appears substantially uniform, whether examined at right angles to the 45 plane of the sheet, or whether the section is taken parallel to the plane of the sheet. To illustrate this, Fig. 6 is taken on an etched portion of the lower side of the sheet, and it will be noted that the crystalline structure 50 is very similar to that of the lower part of Fig. 5, although the plane of the section is at right angles to that of Fig. 5.

55 Summarizing the characteristics of my sheet, then, we find that regardless of thickness, it has a crystalline structure at any one point somewhat similar to that of the ingot of the same material, but varying in size from very fine crystals at one side to comparatively coarse, much larger, crystals at 60 the other side of the sheet. The variation is substantially uniformly progressive from one side of the sheet to the other.

65 By way of illustrating the marked differences of my sheet material, from sheets of the same material made by methods hereto-

fore known and having the usual crystalline structure of such material, as heretofore used in commercial quantities; I have taken this same alloy made in a sheet of the same thickness by the usual process of rolling. 70 The crystal formation of this sheet is illustrated in Fig. 8. It will be noted that the crystalline structure is substantially broken down or obliterated. This rolled sheet is an example of the widely used commercial 75 rolled sheet of lead and its alloys. Fig. 7 is a view showing the structure of mold cast sheets of this same alloy as illustrated in Figs. 1 to 6. The same alloy cast in an ingot or pig, without the influence of any 80 mechanical pressure and allowed to cool naturally, that is simply by radiation is illustrated in Fig. 9. It will be noted that this produces a large pronounced crystalline structure having marked differences from 85 my sheet at any particular point.

As noted in the legends on the drawings, Figs. 7, 8 and 9 are each reproductions of photographs taken at 100 diameters, the same as are Figs. 2 to 6 inclusive.

90 In working toward the end of producing commercial sheet metal more economically than by methods heretofore used, I have sought to produce at the same time a metal having superior properties for the different uses to which it may be put. This I have accomplished by the metal now described, for example, a series of authenticated tests have developed that my sheet of 95 antimony lead used for the purposes of this 100 illustration has very much larger tensile strength than sheets or strips of rolled lead, of the same alloy. For example, the strength tests show that my metal is approximately 105 85% greater in tensile strength and ultimate 110 strength longitudinally of the sheet. I furthermore find that the rolled sheet is very much weaker transversely of the direction of its rolling than it is longitudinally of its direction of rolling, whereas my sheet has 115 the same strength in all directions of the plane of the sheet. That is to say that transversely of the sheet, the tensile strength of my sheet metal is the same as longitudinally of it and it has therefore much higher 120 tensile strength in all directions of the sheet than rolled sheet lead has in the direction of its greatest strength. I also find that a rolled sheet has a tendency to break or split when sharply folded over on itself longitudinally of its direction of rolling, even though it may fail to break or split when sharply folded on itself transversely of the direction of rolling; whereas my sheet, being 125 of uniform characteristics in all directions of the plane of the sheet, has no such pronounced tendency to break or split when folded sharply upon itself along any direction of the plane of the sheet.

130 For use in lining of acid tanks, contain-

ing, for example sulphuric acid or nitrous vitriol, I find my sheets have much greater life than the same alloy when rolled. Tests of applications of sulphuric acid ( $H_2SO_4$ ) specific gravity 1.15 applied for 168 hours disclose that my sheet metal showed no loss of weight, whereas rolled lead similarly treated showed 0.14 per cent loss. Using the same acid specific gravity 1.8 for the same

- 10 length of time and at a temperature of 20 to 25 degrees centigrade, my sheet metal showed about one third as much loss as rolled metal of the same alloy. The same was true of a nitrous vitriol test. The use 15 of this metal for lining of acid tanks is very advantageous, offering a cheaper metal of higher resisting qualities and greater length of life in service.

It is to be understood that the illustration 20 of antimony lead as embodying this invention or discovery, is not to be taken as a limitation of this invention to this material, as practice has demonstrated that many other metals are included within the scope 25 of this invention. The characteristics, both crystalline and physical properties, of other metals having melting points of sufficiently low temperature as to be feasibly manufactured by my method, are very similar.

30 For convenience, I may mention in this specification that a method of manufacturing the metal embodying the characteristics of this invention has been found to result from the use of stationary and relatively 35 moving members between which the molten metal is caused to flow and pass therefrom in its frozen state. The temperatures of the two mold members are so governed as to secure a relative difference between them, 40 causing one side of the sheet to cool somewhat more rapidly than the other, while on the slower cooling side (i. e., higher temperature) the cooling is such as to freeze the material just as it passes from between the 45 mold members.

What I claim is:

1. A sheet of metal of predetermined thickness having uniform surfaces and having before any further treatment a different

crystalline structure at and near one side of 50 the sheet than the structure at and near the other side of the sheet.

2. A sheet of metal cast but not otherwise treated and of the same constitution throughout but having a variation in crystalline formation ranging from coarse crystals at one side of the sheet to fine crystals 55 at the other side of the sheet.

3. A sheet of cast metal of the same constitution throughout having defined regular opposite surfaces and before further treatment consisting of a fine grain crystalline structure at one side and a comparatively coarse grain crystalline structure at 60 the other.

4. A cast sheet of metal or metal alloy of the same constitution throughout but having a variation in crystalline formation so that one side of the sheet are coarse grains or crystals, at the other side of the sheet are 70 fine grains or crystals, while intermediate the two sides is an intermediate size of grains or crystals.

5. A cast thin sheet of metal having one side structurally different from the other 75 and having a tensile strength greater in any line of the plane of the sheet than rolled sheet of the same composition and thickness is in the line of its greatest strength.

6. A cast sheet of metal formed in a continuous strip and having a crystalline structure throughout and having a tensile strength transversely of the strip equal to that longitudinally of the strip.

7. A cast sheet of metal formed in a continuous strip and having no apparent grain in any direction of the material as compared to the grain of a rolled sheet.

8. A cast metal sheet formed in a continuous strip of indefinite length and having a 90 crystalline structure uniform longitudinally of the sheet, though varying from large to fine crystals from one plane surface of the sheet to the other.

In testimony whereof, I hereunto affix my 95 signature.

CLARENCE W. HAZELETT.